

March 3, 1959

2,875,896

A. W. LAST ET AL  
PROCESS OF CONCENTRATING COLUMBIUM MINERALS  
BY FROTH FLOTATION  
Filed Oct. 10, 1957



INVENTOR.

ARTHUR W. LAST  
KENT F. MARQUARDSON

BY  
*J. R. Mallinckrodt and*  
*Philip A. Mallinckrodt*  
ATTORNEYS

**PROCESS OF CONCENTRATING COLUMBIUM  
MINERALS BY FROTH FLOTATION**

Arthur W. Last and Kent F. Marquardson, Salt Lake City, Utah, assignors to Kennecott Copper Corporation, New York, N. Y., a corporation of New York

Application October 10, 1957, Serial No. 689,435

14 Claims. (Cl. 209—166)

This invention relates to the art of froth flotation for the selective recovery of specific minerals from their ores. It has particular reference to the recovery of columbium minerals from the ores in which they are found.

The metallic element niobium, or columbium as it is commonly called by metallurgists, has been known well over a hundred years. It occurs in various mineral forms.

There are vast deposits of columbium ores that have been left unworked for the lack of any effective and economical process for separating the valuable minerals from the gangue materials with which they are associated in the natural ore deposits. Certain ores containing the mineral columbite are being worked in instances where separation of the columbite by gravity means, electrostatic means, or by magnetic means has proven economically feasible. However, such separation procedures have not been economical in their application to ores containing other columbium minerals, such as pyrochlore, perovskite, nioclate, betafite, etc.

No successful flotation process has to our knowledge yet been reported for the selective flotation and recovery of columbium minerals. There has hitherto been no known reagent capable of floating such minerals on a selective basis.

We have found that columbium minerals may be effectively and economically floated from gangue constituents of an ore by the use of a reagent selected from a particular group of chemical compounds, serving as a collector selective to such columbium minerals. The group of chemical compounds consists of a hydroxy-quinoline, specifically, 8-quinolinol, commonly known as "oxine," and mono-lower-alkyl-substituted 8-quinolinols.

While 8-quinolinol is well known as a chemical compound, it is normally used in highly purified form in the chemical art as an analytical reagent. The only instances where 8-quinolinol has even been tried as a flotation reagent is in connection with certain academic investigations concerned with abstract flotation theory. In such instances, the materials involved were merely artificial mixtures containing solely zinc, iron, tungsten, and titanium minerals. Such experiments have evoked little interest, and have given no indication that the particular reagent has any effectiveness as applied to columbium.

In accordance with the present invention, the ore is finely ground in a manner customary in conventional flotation practice, and is subjected to agitation and aeration, as an aqueous pulp, in the presence of the particular reagent specified. The columbium minerals are effectively collected in the froth, to yield a columbium concentrate.

A principal object of the present invention is to provide a froth flotation process whereby columbium minerals may be effectively recovered from their ores on a selective basis as respects other constituents of such ores.

Another object is to minimize reagent consumption and expense.

A principal feature of the invention is the agitation and aeration of a flotation pulp of columbium ore in the presence of 8-quinolinol or a mono-lower-alkyl-substituted 8-quinolinol thereof, serving as a collecting agent for 5 the columbium mineral or minerals in the ore to the exclusion of other constituents of the ore.

A significant feature in the minimizing of reagent expense is the use of an impure reaction product, rather than the chemically pure analytical reagent.

- 10 Another feature useful in minimizing reagent consumption is the reclaiming of the reagent-bearing solution from the final flotation pulp, and the use of same in preparing the initial flotation pulp for a subsequent run. This is advantageously done in connection with still 15 another feature of the invention, namely, preliminary treatment of the ore for the elimination of various gangue constituents, particularly calcite, apatite, mica, magnetite, and iron sulfide minerals.
- 20 In the preferred practice incorporating all of the above features, the ore pulp resulting from preliminary treatment for gangue elimination is dewatered. It is then re-pulped in recovered reagent-bearing solution prior to undergoing the significant froth flotation stage of the process.
- 25 Further objects and features of the invention will become apparent as the description proceeds with respect to specific procedures and test results.

Our work has shown that 8-quinolinol ( $C_9H_7NO$ ) having the formula:



is an active flotation reagent for columbium minerals when used either in the form of the chemically pure analytical reagent or in a crude form obtained as an impure reaction product of a known procedure.

This has been demonstrated by numerous laboratory tests, typified by those set forth herebelow:

**COMPARATIVE TESTS AS BETWEEN PURE AND CRUDE REAGENT**

- 45 In this series of tests, respective 1,000 gram charges of a low grade, carbonatite type, columbium ore from the province of Quebec, Canada, containing less than 0.6 percent columbium oxide ( $Cb_2O_5$ ) in the form of the minerals pyrochlore, perovskite, and others not yet definitely identified nor classified but believed to include at least both nioclate and betafite, were ground to 90 percent minus 200 mesh. They were carefully deslimed, and were individually conditioned with the quantity of 50 the reagent specified in the following tabulated test data and with 20 drops (0.6 gram) of burner oil, i. e. domestic fuel oil, for approximately one minute. They were then individually subjected to agitation and aeration in a laboratory flotation machine, and respective froth 55 concentrates of the columbium minerals were recovered.

60 As indicated in the tabulation, the reagent was used in its chemically pure form for one of the tests and in a crude form for the others.

65 The crude reagent was prepared according to the procedure set forth in the treatise "Organic Analytical Reagents," vol. 1, 1947, D. Van Nostrand Co., Inc., by mixing 5 grams of o-nitrophenol, 8.3 grams of o-aminophenol, and 18 grams of glycerol in a 500 ml. flask, and slowly adding 8.2 ml. of concentrated  $H_2SO_4$ , the flask being fitted with a reflux condenser, and the mixture being boiled gently for five hours. Following cooling, the resulting solution was diluted to a volume of 250 ml.

## Tests.—Rougher concentrate

| Reagent                                                       | Weight, percent | Cb <sub>2</sub> O <sub>5</sub> , percent | Recovery, percent |
|---------------------------------------------------------------|-----------------|------------------------------------------|-------------------|
| (1) 2 g. C. P. 8-quinolinol                                   | 36.8            | 1.49                                     | 90.6              |
| (2) 60 ml. crude 8-quinolinol solution                        | 33.0            | 1.66                                     | 84.5              |
| (3) 80 ml. crude 8-quinolinol solution                        | 44.0            | 1.37                                     | 93.9              |
| (4) 80 ml. crude 8-quinolinol solution (reflux time 10 hours) | 39.7            | 1.18                                     | 90.7              |

We have also found that reagent consumption can be reduced by treating the ore for removal of various gangue minerals prior to flotation for recovery of the columbium minerals. A typical test is reported herebelow:

## PRELIMINARY UPGRADING BY REMOVAL OF GANGUE CONSTITUENTS

This was a locked cyclic test, wherein, for each cycle, various gangue constituents were removed by conventional techniques indicated in the optional portion of the flow sheet of the accompanying drawing.

A charge of 4,000 grams of the same carbonatite type, columbium ore was prepared for each cycle as in the foregoing tests, and was made into an aqueous pulp in accordance with conventional practice. Such aqueous pulp was subjected to flotation with a fatty acid collector reagent to remove calcite and apatite. The froth concentrate was passed to waste, and the tailings were subjected to sulfide flotation utilizing a sulfonated petroleum oil and a xanthate collector as reagents. The froth concentrate was passed to waste, and the tailings subjected to magnetic separation for the removal of magnetite.

The resulting upgraded ore pulp (from 0.6 percent Cb<sub>2</sub>O<sub>5</sub> to 2.36 percent Cb<sub>2</sub>O<sub>5</sub>) was deslimed, and the deslimed pulp conditioned with 2 grams of C. P. 8-quinolinol and 1.5 grams of burner oil for flotation.

Agitation and aeration of the so conditioned pulp in a laboratory flotation machine resulted in a columbium-bearing froth, which was cleaned twice by further flotation of the same character. The cleaner tailings were added to the subsequent batch of ore pulp in accordance with closed cycle practice. The metallurgical results were as follows:

|                                         | Weight, percent | Cb <sub>2</sub> O <sub>5</sub> , percent | Distribution, percent |
|-----------------------------------------|-----------------|------------------------------------------|-----------------------|
| Calculated Headings (Upgraded Ore Pulp) |                 |                                          |                       |
| Concentrate                             | 21.4            | 9.72                                     | 88.0                  |
| Tailing                                 | 78.6            | .36                                      | 12.0                  |

In addition to the above, we have found that a large portion of the comparatively expensive reagent can be recovered and reused by reclaiming the solution from the flotation pulp. This is the presently preferred procedure, and is advantageously carried out in connection with the above-described preliminary treatment for removal of various gangue constituents from the ore, all as indicated by the flow sheet of the accompanying drawing.

A typical test conforming to such flow sheet appears herebelow:

## RECOVERY OF REAGENT-BEARING SOLUTION

For this cyclic test, 1,000 gram batches of the same carbonatite type, columbium ore, prepared as in the foregoing tests, were deslimed and upgraded by the afore-described mica and iron sulfide flotation and by removal of magnetite. In this instance, the pulp was not treated for removal of calcite and apatite.

The upgraded ore pulp was filtered, and the filter cake was used in the preparation of the aqueous pulp for the columbium flotation. The solution employed for this repulping operation was prepared initially from crude reagent obtained in the same manner as for the first series of tests, although, here, the reflux time was ten hours

(as in the fourth of the foregoing tests) instead of five.

Six liters of solution were prepared from 150 ml. of the crude reagent. This supplied all dilution and wash water used during the flotation procedure, as well as the aqueous phase of the flotation pulp.

Agitation and aeration of the reagent-bearing pulp resulted in a columbium-bearing froth concentrate. The froth and tailings were separately filtered, and the respective filtrates were returned to the original solution. An additional 25 ml. of crude reagent was then added to the solution, and the procedure was repeated.

In all, the procedure was carried out a total of six times. The recovery and grade of concentrates from the sixth cycle (after equilibrium was achieved) are tabulated as follows:

## Rougher concentrate

| Reagent                                          | Weight, percent | Cb <sub>2</sub> O <sub>5</sub> , percent | Recovery, percent |
|--------------------------------------------------|-----------------|------------------------------------------|-------------------|
| 25 ml. crude 8-quinolinol solution (sixth cycle) | 40.0            | 1.36                                     | 92.8              |

The difference in reagent consumption between the straight flotation process using 8-quinolinol as a reagent and the more preferred practice of upgrading prior to flotation, coupled with recycling the liquid phase of the tailings and froth concentrate from the 8-quinolinol flotation, is well demonstrated by comparing Test No. 4 of the first series of tests with the last test above. It will be seen that comparable recovery was made in the latter instance with only 25 ml. of the crude reagent solution as compared with 80 ml. for the former.

In the course of our work, many flotation tests were made using various conventional reagents in an effort to float columbium minerals. However, none of these yielded economic recovery. Accordingly, no comparative tests as between the reagent here disclosed and other reagents are presented.

Our tests have shown that the 8-quinolinol reagent, whether in chemically pure or crude form, is effective in acid, neutral, or basic pulps. In such tests, however, recovery has fallen off considerably in the extremes of pH range. Accordingly, it is preferred that this flotation process be carried out with a near neutral pulp.

The 8-quinolinol reagent has proven to have natural frothing properties, which makes it unnecessary to add any other frothing reagent in many instances in which the process is used. It should be kept in mind, however, that the natural frothing properties may be supplemented wherever found desirable by addition of a conventional frothing agent, such as pine oil.

We have conducted tests on many different types of ores containing a variety of columbium minerals. These tests indicate that our process is effective on columbium minerals in general.

The following examples detail representative tests showing ratios of concentration of 1 to 12.1, 1 to 41.7, and 1 to 9.5, respectively:

## EXAMPLE NO. 1

Two thousand grams of the carbonatite-type ore utilized in the previous tests were ground to approximately 90 percent minus 200 mesh, deslimed, the iron sulfide minerals removed from the ore pulp by flotation using xanthate collector, and the magnetite removed magnetically. The ore pulp was then filtered, split into two equal parts, and each part was individually re-pulped in a laboratory flotation machine, conditioned with 2.5 grams of 8-quinolinol, and a froth concentrate recovered. The tailings were combined for assay, and the froth concentrates were combined, conditioned with 0.5 gram of 8-quinolinol, and a froth concentrate recovered by flotation. The concentrate was then recleaned three times by flotation, using the solution recovered (by filtration) from the tailings of the previous step for dilution water.

**5**  
*Test results*

| Product             | Weight, percent | Cb <sub>2</sub> O <sub>5</sub> , percent | Distribution, percent |
|---------------------|-----------------|------------------------------------------|-----------------------|
| Rougher Tailing     | 60.93           | 0.04                                     | 3.67                  |
| 1st Cleaner Tailing | 22.01           | 0.22                                     | 7.28                  |
| 2nd Cleaner Tailing | 6.09            | 0.48                                     | 4.39                  |
| 3rd Cleaner Tailing | 1.94            | 0.62                                     | 1.81                  |
| 4th Cleaner Tailing | 0.79            | 0.85                                     | 1.01                  |
| Concentrate         | 8.24            | 0.60                                     | 81.84                 |
| Calculated Heading  | 100.00          | 0.66                                     | 100.00                |

## EXAMPLE NO. 2

One thousand grams of a pyrochlore-bearing granite from Nigeria were ground at 67 percent solids for twenty-three minutes in a laboratory ball mill. The resultant pulp was deslimed, filtered, re-pulped in a laboratory flotation machine, conditioned with four grams of 8-quinolinol, and a froth concentrate removed. The froth concentrate was cleaned twice by flotation.

*Test results*

| Product             | Weight, percent | Cb <sub>2</sub> O <sub>5</sub> , percent | Distribution, percent |
|---------------------|-----------------|------------------------------------------|-----------------------|
| Rougher Tailing     | 73.83           | 0.06                                     | 21.93                 |
| 1st Cleaner Tailing | 16.21           | 0.19                                     | 15.26                 |
| 2nd Cleaner Tailing | 7.56            | 0.33                                     | 12.33                 |
| Concentrate         | 2.40            | 4.25                                     | 50.49                 |
| Calculated Heading  | 100.00          | 0.20                                     | 100.00                |

## EXAMPLE NO. 3

Twenty-five grams of columbite from Nigeria and one thousand grams of a quartz-monzonite rock were combined and ground for ten minutes in a laboratory ball mill. The resultant pulp was deslimed, and the sulfide minerals removed by flotation with Minerec "A" and burner oil as collectors. The pulp was then conditioned with two grams of 8-quinolinol, and a froth concentrate recovered. The concentrate was cleaned once by flotation.

*Test results*

| Product             | Weight, percent | Cb <sub>2</sub> O <sub>5</sub> , percent | Distribution, percent |
|---------------------|-----------------|------------------------------------------|-----------------------|
| Rougher Tailing     | 68.32           | 0.07                                     | 2.36                  |
| 1st Cleaner Tailing | 21.17           | 1.25                                     | 13.06                 |
| Concentrate         | 10.51           | 16.3                                     | 84.58                 |
| Calculated Heading  | 100.00          | 2.02                                     | 100.00                |

It will be obvious that various other elements, such as uranium, that are intimately associated with the columbium minerals will also be recovered by this process.

Comparative tests have been carried out, as follows:

*Test No. 1 (8-quinolinol)*

Five hundred grams of a low grade carbonate type ore containing the columbium minerals Pyrochlore and Perovskite and upgraded by removal of calcite and apatite, by desliming, and by removal of iron sulfide and magnetite were subjected to a batch flotation procedure involving flotation at pH 7.2 to 8.0 for ten minutes in the presence of two and one-half grams of 8-quinolinol. The rougher froth concentrate obtained was cleaned by re-flotation, with the following results:

| Product             | Weight, percent | Cb <sub>2</sub> O <sub>5</sub> , percent | Distribution, percent |
|---------------------|-----------------|------------------------------------------|-----------------------|
| Cleaner Concentrate | 4.74            | 10.36                                    | 31.00                 |
| Cleaner Tailing     | 22.35           | 3.39                                     | 47.83                 |
| Rougher Tailing     | 72.91           | 0.46                                     | 21.17                 |
| Calculated Feed     | 100.00          | 1.58                                     | 100.00                |

**6***Test No. 2 (2-methyl-8-quinolinol)*

The procedure here was identical with that of the foregoing test, except 3.5 grams of 2-methyl-8-quinolinol (8-hydroxyquinaldine) were used as the collector reagent. Results were as follows:

| Product             | Weight, percent | Cb <sub>2</sub> O <sub>5</sub> , percent | Distribution, percent |
|---------------------|-----------------|------------------------------------------|-----------------------|
| Cleaner Concentrate | 6.60            | 9.21                                     | 30.82                 |
| Cleaner Tailing     | 24.68           | 4.07                                     | 40.90                 |
| Rougher Tailing     | 68.72           | 0.53                                     | 18.28                 |
| Calculated Feed     | 100.00          | 1.98                                     | 100.00                |

*Test No. 3 (4-methyl-8-quinolinol)*

The procedure here was identical with the foregoing tests, except 2.0 grams of 4-methyl-8-quinolinol were used as the collector reagent. Results were as follows:

| Product               | Weight, percent | Cb <sub>2</sub> O <sub>5</sub> , percent | Distribution, percent |
|-----------------------|-----------------|------------------------------------------|-----------------------|
| Reclaimer Concentrate | 3.18            | 19.3                                     | 34.70                 |
| Reclaimer Tailing     | 7.01            | 5.24                                     | 20.77                 |
| Cleaner Tailing       | 43.10           | 1.60                                     | 38.99                 |
| Rougher Tailing       | 46.71           | 0.21                                     | 5.54                  |
|                       | 100.00          | 1.77                                     | 100.00                |

*Test No. 4 (6-methyl-8-quinolinol)*

The procedure here was identical with the foregoing tests, except 2.0 grams of 6-methyl-8-quinolinol were used as the collector reagent. Results were as follows:

| Product               | Weight, percent | Cb <sub>2</sub> O <sub>5</sub> , percent | Distribution, percent |
|-----------------------|-----------------|------------------------------------------|-----------------------|
| Reclaimer Concentrate | 7.61            | 5.59                                     | 26.16                 |
| Reclaimer Tailing     | 16.30           | 2.63                                     | 26.36                 |
| Cleaner Tailing       | 38.04           | 1.77                                     | 41.40                 |
| Rougher Tailing       | 38.05           | 0.28                                     | 6.08                  |
|                       | 100.00          | 1.63                                     | 100.00                |

Of the several reagents used in the above series of tests, only 8-quinolinol is readily available. It was possible to purchase the reagent for Test No. 2 from Eastman Kodak Company, but the reagents for Tests No. 3 and 4 were synthesized in the laboratory.

This application constitutes a continuation-in-part of our copending application Serial Number 612,849, filed Sept. 28, 1956, entitled "Process of Concentrating Niobium Minerals by Froth Flotation," which has been found to be allowable but which has been abandoned in favor of the present application.

We claim:

1. In a process of froth flotation for the separation of columbium minerals from other constituents of a columbium ore, the steps of agitating and aerating an aqueous pulp containing said columbium ore and 8-quinolinol, the latter serving as a collector reagent selective to columbium minerals; and recovering the resulting froth as a columbium concentrate.
2. The process of claim 1, wherein the said steps are preceded by pre-concentration treatment of an aqueous pulp of the ore.
3. The process of claim 2, wherein the procedure is carried out on a cyclic basis, and, following the said steps of each cycle, at least the tailings are treated for recovery of their reagent-bearing liquid phase; wherein the upgraded pulp is treated for removal of its liquid phase; and wherein the solid phase of said upgraded pulp is re-pulped with the recovered reagent-bearing liquid phase.
4. The process of claim 3, wherein the 8-quinolinol is an impure reaction product.

5. The process of claim 1, wherein the aqueous pulp also contains a neutral petroleum oil.

6. The process of claim 1, wherein the 8-quinolinol is an impure reaction product.

7. The process of claim 1, wherein at least the tailings resulting from the said steps are treated for recovery of their reagent-bearing liquid phase; and wherein the said liquid phase is used in pulping additional ore for said process.

8. The process of claim 1, wherein the said steps are preceded by flotation of sulfide minerals from an aqueous pulp of the ore, for upgrading said ore.

9. In a process of froth flotation for the separation of columbium minerals from other constituents of a columbium ore, the steps of agitating and aerating an aqueous pulp containing said columbium ore and a collector reagent selected from the group consisting of 8-quinolinol and mono-lower-alkyl-substituted 8-quinolinols; and recovering the resulting froth as a columbium concentrate.

10. The process of claim 9, wherein the said steps are preceded by pre-concentration treatment of an aqueous pulp of the ore.

5 11. The process of claim 10, wherein the procedure is carried out on a cyclic basis, and, following the said steps of each cycle, at least the tailings are treated for recovery of their reagent-bearing liquid phase; wherein the upgraded pulp is treated for removal of its liquid phase; and wherein the solid phase of said upgraded pulp is re-pulped with the recovered reagent-bearing liquid phase.

10 12. The process of claim 9, wherein the aqueous pulp also contains a neutral petroleum oil.

15 13. The process of claim 9, wherein at least the tailings resulting from the said steps are treated for recovery of their reagent-bearing liquid phase; and wherein in the said liquid phase is used in pulping additional ore for said process.

14. The process of claim 9, wherein the said steps are preceded by flotation of sulfide minerals from an aqueous pulp of the ore, for upgrading said ore.

20 **References Cited in the file of this patent**

Oxine and Its Derivatives, Hollingshead, vol. II, 594-596, 1954.